

Aug. 16, 1927.

J. L. DRAKE

1,639,452

DRAWING SHEET GLASS

Filed May 15, 1924

2 Sheets-Sheet 1



FIG. 5.

FIG. 7.



INVENTOR.  
John L. Drake  
BY C. A. Crowley  
ATTORNEY.

Aug. 16, 1927.

**1,639,452**

J. L. DRAKE

DRAWING SHEET GLASS

Filed May 15. 1924

2 Sheets-Sheet 2



INVENTOR.  
John L. Drake  
BY C. A. Powley  
ATTORNEY.

Patented Aug. 16, 1927.

1,639,452

# UNITED STATES PATENT OFFICE.

JOHN L. DRAKE, OF CHARLESTON, WEST VIRGINIA, ASSIGNOR TO THE LIBBEY-  
OWENS SHEET GLASS COMPANY, OF TOLEDO, OHIO, A CORPORATION OF OHIO.

## DRAWING SHEET GLASS.

Application filed May 15, 1924. Serial No. 713,390.

This invention relates to the art of drawing sheet glass, and more particularly to an improved process and apparatus for maintaining the width of the sheet and imparting lateral tension to the sheet during the sheet forming period.

In the Colburn system of drawing sheet glass as set forth for example in the patent to I. W. Colburn, 1,248,809, granted Dec. 10, 1917, the glass sheet is continuously drawn upward from the surface of a shallow pool of molten glass, and after the sheet form is substantially established, but while the sheet is still somewhat plastic, it is deflected about a cooled bending roller into the horizontal plane and thence carried away through suitable drawing and flattening mechanism into the leer. A pair of small edge-forming rollers grip each sheet 15 edge at its source. These rollers are positively driven at a peripheral speed considerably less than the speed at which the glass is drawn about the bending roller. Thus these edge rollers function not only to positively feed glass upwardly from the molten pool into the edges of the sheet, but also hold back on the edge portions of the vertical run of the sheet so as to establish a stretching tension therein. In this way the 20 rollers function, in cooperation with the bending roll, to hold the sheet to a substantially constant width, and counteract the sheet's natural tendency to narrow away at its source. It will be noted however, that 25 there is no positive means exerting lateral tension on any portion of the vertical run of the sheet between the sheet source and the bending roller, and the sheet due to its natural tendency to contract when cooling, and 30 also due to the longitudinal elongation to which it is subjected during this period, becomes several inches narrower at the bending roller than it is at its source. It is also believed that the absence of lateral tension 35 in the sheet during this period is one cause of certain waves or inequalities in sheet thickness sometimes present in the drawn sheet.

According to the present invention a second pair of edge-gripping rollers are positioned in engagement with the edge of the sheet at a point in its vertical run intermediate the source and the bending member. These rollers are positively driven at a

speed intermediate that of the edge forming rollers and the bending roller, that is their peripheral speed is faster than that of the edge-forming rollers, but slower than that of the bending roller or the sheet drawing means. In this way a longitudinal tension is maintained in that portion of the sheet edge between the two pairs of edge-gripping rollers, and at the same time longitudinal tension is maintained between the intermediate edge-gripping rollers and the bending roller. Due to these variations in sheet engaging speeds, and the longitudinal sheet tension resulting therefrom, the sheet may be continuously held between the upper pairs of rollers and forced to follow a more nearly vertical path than is the case when these auxiliary rollers are not used. In other words, the tendency for the sheet to contract immediately above the edge-forming rollers is resisted to such an extent that the finished sheet will be several inches wider than was formerly the case, and at the same time the sheet during its formative period will be subjected to a continuous lateral stress through the zone immediately above its source, thus tending to eliminate waves or other inequalities that might result from the lack of adequate lateral tension.

The objects and advantages of the invention will be better understood from the following detailed description of one approved form of the apparatus.

In the accompanying drawings:

Fig. 1 is a transverse vertical section through the receptacle containing the pool of molten glass, the sheet edge drawing and bending members being shown in elevation.

Fig. 2 is a similar elevation, on an enlarged scale, of one set of edge-forming and stretching members.

Fig. 3 is an end elevation of the mechanism shown in Fig. 2.

Fig. 4 is a plan view of one of the upper sets of edge-gripping rollers and the supporting and driving mechanism therefor.

Fig. 5 is an enlarged elevation of the driving gears whereby the two sets of rollers are driven simultaneously at the desired speed. This view is taken substantially on the line 5-5 of Fig. 1.

Fig. 6 is a longitudinal vertical section illustrating diagrammatically the relative

positions of the sheet-drawing, bending and edge-forming members. This view is taken substantially on the line 6—6 of Fig. 1.

Fig. 7 is a detail showing a modified form 5 of the edge-rollers.

The glass sheet 1 is drawn upwardly from the pool of molten glass 2 in receptacle 3, and then while still somewhat plastic is bent about the cooled bending roller 4 into a horizontal plane. It is then drawn away over 10 suitable supporting rollers such as 5 into a drawing and flattening mechanism 6. This mechanism 6 furnishes the drawing force for continuously pulling the glass sheet 1 from 15 the molten source 2.

Gripping each edge of the sheet 1 at its source is a pair of driven rollers 7, usually provided with a roughened or knurled surface to insure a positive grip upon the molten 20 glass passing therebetween. These rollers 7 are mounted on the inner ends of suitable rotary shafts 8. The auxiliary edge-drawing rollers 9, forming the particular subject-matter of the present invention, may have 25 substantially the same form as rollers 7 and are mounted at the inner ends of shafts 10 similar in all respects to the shafts 8.

The supporting and driving means for 30 each pair of shafts 8 and 10, at either side of the sheet, are substantially identical, and a description of one will suffice for all. One of each pair of shafts 8 or 10 is journaled in a fixed bearing bracket 11 carried by or 35 formed on a supporting plate 12. The other shaft 8 or 10 of the pair is journaled in a similar bearing 13 pivoted as at 14 in the supporting plate 12 so that the roller 7 or 9 carried thereby may be swung toward or from its companion roller. A spring 15 40 whose compression is adjustable by means of screw 16 is mounted between the bearings 11 and 13 so as to normally force the pair of rollers 7 or 9 toward one another. A handle 17 secured to the side of the movable bearing 13 forms a convenient means for swinging 45 the movable roller away from its companion roller to enable the sheet to be engaged therebetween. When the handle 17 is released, the spring 15 will force the two 50 rollers toward one another in yielding contact with the sheet edge. The supporting plate 12 is provided with a flange 18 at one edge engaging a complementary recess in a supporting frame 19 carried by stationary 55 beam 20 at the side of the machine. Clamping screws 21 extending through the opposite side of frame 19 engage the opposite edge 22 of plate 12 to hold the same in any desired fixed position. By loosening the 60 screws 21 the roller assembly may be moved in or out with relation to the edge of glass sheet 1.

A continuous flow of water or other cooling fluid passes in through pipe 23, which 65 extends inwardly through pipe 8 to the in-

terior of the roller 7, this water then flowing back through pipe 8 and around pipe 23, and out through the exit pipe 24. In this way the roller 7 and pipe 8 are continuously filled with a constantly renewed supply of 70 cooling fluid. This protects the roller and shaft from the intense heat to which they are subjected, and at the same time exerts a cooling action on the edge portions of the sheet which assists in the sheet formation. 75 It will be understood that each of the shafts 8 and 10 and rollers 7 and 9 is provided with a similar individual cooling system.

A bevel gear 25 secured to one shaft 8 meshes with and is driven by a similar bevel gear 26 on a stub-shaft 27 driven through universal joint 28 from a drive shaft 29. A pair of similar intermeshing spur gears 30, one secured to each shaft 8, serve to drive the two shafts and the rollers 7 at the same 80 speed but in opposite directions. A spur gear 31 secured to one of the shafts 8 meshes with an intermediate spur gear 32, which in turn meshes with a gear 33 secured to one of the shafts 10. Intermediate gear 32 is 85 carried in a frame 34 supported at its lower end on the pair of shafts 8. The bearing 35 for one of the shafts 8 is 90 slidable in slots 36 in the main body portion of frame 34 and permits shafts 8 to be moved toward or from one another in adjusting the 95 position of roller 7. A pair of intermeshing spur gears 37, one of which is secured to each shaft 10 serve to drive the two shafts 10 at the same speed but in opposite directions. The proportions of several gears 31, 32 and 33 will be so designed that shafts 10 will be rotated at a somewhat greater speed 100 than shafts 8. In this way the peripheral speed of the upper pair of rollers 9 will be 105 greater than the peripheral speed of the lower edge-forming rollers 7.

In the normal operation of sheet drawing machines of this type, as disclosed in the Colburn patent referred to hereinabove, the 110 edge-forming rollers 7 are driven at a considerably slower peripheral speed than the linear speed imparted to the body of the sheet as a whole by the main drawing means 6. In this way the positively driven rollers 115 7 feed molten glass up into the sheet edges from molten pool 2 at a rather slow rate, and subsequently this edge glass is stretched or elongated during its vertical passage up to the bending roll 4 until the edge portions 120 of the sheet have reached the speed imparted to the entire sheet body by the drawing mechanism 6. In this way the final width of the continuous sheet is maintained practically constant, but the sheet narrows up 125 considerably in its passage from edge-forming rollers 7 to bending roll 4 as indicated by the dotted lines 38 in Fig. 1.

When the supplemental edge-drawing rollers 9 are used the still plastic sheet is 130

stretched out by means of hooks or other suitable tools until it engages between the driven rollers 9. Since these rollers 9 are driven at a greater speed than rollers 7 a 5 longitudinal tension or drawing force will be exerted on that portion of the sheet edge between the rollers 7 and 9 and the sheet will remain in engagement with both pair of rollers. At the same time since rollers 9 10 are driven slower than the drawing mechanism 6, there will also be a stretching tension between the rollers 9 and the bending roller 4. It has been discovered that as a result of this drawing operation, the glass sheet 1 will 15 maintain a practically constant width from its source up to the bending roller 4, at which point it has become set to such an extent that there is very little further lateral contraction. At the same time the additional 20 lateral tension imparted to the sheet during its formative period tends to eliminate the waves or other surface inequalities which otherwise might be present in the sheet.

It has been noted that when the additional 25 edge-rollers 9 are used, the "meniscus" 39, or mass of glass drawn up from the molten pool at the sheet source is thicker and rises to a greater height than was previously the case. Thus in some manner, these auxiliary 30 rollers function to actually draw a greater amount of glass up into the sheet, and do not merely stretch to a greater width the mass of glass drawn up by the drawing mechanism 6 and edge-rollers 7, although the sheet is at 35 the same time subjected to a greater lateral tension than was previously the case.

The distance of rollers 9 above rollers 7 may be varied, but should not be sufficient to bring the rollers 9 outside of the initial 40 forming zone of the sheet. The sheet 1 should still remain sufficiently plastic to be positively engaged by the knurled surface of rollers 9.

The rollers 7 and 9 need not necessarily 45 be constructed of the exact cylindrical form shown in Figs. 1, 2 and 4 although this form has been operated successfully. The lower rollers may be shaped as shown at 40 in Fig. 7, so as to form a thicker edge or bead on the sheet. The upper rollers may also be given this configuration, or if cylindrical as at 9, will have a thicker mass of plastic glass to engage, thus insuring a more positive grip 50 on the sheet. Many other forms of sheet-gripping surfaces might be given to these rollers without departing from the principles 55 of this invention.

Claims:

1. In the art of drawing sheet glass from 60 a mass of molten glass, the method consisting in applying longitudinal drawing forces to the sheet edges only at the sheet source, applying supplemental drawing forces to the sheet edges only at a greater drawing speed 65 at points beyond the sheet source, and sub-

sequently applying a still faster drawing force to the entire body of the sheet.

2. In an apparatus for drawing sheet glass, a plurality of pairs of edge-gripping rollers engaging each edge of the sheet, and 70 means for simultaneously driving the pairs of rollers at different speeds, the rollers most remote from the sheet source having the greatest speed.

3. In an apparatus for drawing sheet 75 glass, a container for a supply of molten glass, a bending roller about which the plastic sheet is deflected, a pair of edge-forming rollers engaging each sheet edge at its source, the edge rollers being driven at a peripheral speed less than that of the bending roller, pairs of edge rollers engaging the sheet edge 80 between the edge-forming rollers and the bending roller and means for positively driving these intermediate rollers at a peripheral speed greater than that of the edge-forming rollers but less than that of the bending roller.

4. In sheet glass apparatus, means for 90 drawing a sheet from a mass of molten glass, a plurality of pairs of edge gripping rollers engaging each edge of the sheet, the pairs of rollers at each edge being rotated at different relative speeds, while the corresponding rollers in each pair are driven at substantially the same speed.

5. In sheet glass apparatus, means for 95 drawing a sheet from a mass of molten glass, pairs of rolls arranged at each edge of the sheet and engaging the same, and means for driving the pairs of rolls at different speeds, the corresponding rolls in each pair being driven at the same speed.

6. In sheet glass apparatus, means for 100 drawing a sheet from a mass of molten glass, pairs of rolls arranged at each edge of the sheet and engaging the same, and means for retarding the pairs of rolls in a manner that their peripheral speeds will be different, the peripheral speed of corresponding rolls in 105 each pair being the same.

7. In sheet glass apparatus, means for 110 drawing a sheet from a mass of molten glass, pairs of rolls arranged at each edge of the sheet and engaging the same, means for retarding the pairs of rolls in a manner that their peripheral speeds will be different, the peripheral speed of corresponding rolls in 115 each pair being the same, and means for controlling the temperature of the rolls.

8. In sheet glass apparatus, means for 120 drawing a sheet from a mass of molten glass, pairs of rolls arranged at each edge of the sheet and engaging the same, the lower pair of rolls being arranged at the formative portion of the edge, and the upper pair of rolls being arranged at substantially the point where the edge normally moves inwardly of the sheet.

9. In sheet glass apparatus, means for drawing a sheet from a mass of molten glass, pairs of rolls arranged at each edge of the sheet and engaging the same, the lower pair of rolls being arranged at the formative portion of the edge, and the upper pair of rolls being arranged at substantially the point where the edge normally moves inwardly of the sheet, and means for driving the upper rolls in a manner that they will have a relatively greater peripheral speed than the lower rolls.

10. In sheet glass apparatus, means for drawing a sheet from a mass of molten glass, pairs of rolls arranged at each edge of the sheet and engaging the same, the lower pair of rolls being arranged at the formative portion of the edge, and the upper pair of rolls being arranged at substantially the point where the edge normally moves inwardly of the sheet, and means for controlling the temperature of said rolls.

11. In sheet glass apparatus, means for drawing a sheet from a mass of molten glass, upper and lower rolls arranged at each edge of the sheet and engaging the same, the upper roll having a peripheral speed relatively greater than that of the lower roll.

12. In sheet glass apparatus, means for drawing a sheet from a mass of molten glass, upper and lower rolls arranged at each edge of the sheet and engaging the same, and means for retarding both rolls in a manner that their peripheral speeds will be different.

13. In sheet glass apparatus, means for drawing a sheet from a mass of molten glass, upper and lower rolls arranged at each edge of the sheet and engaging the same, the lower roll being arranged at the formative portion of the edge and the upper roll being arranged at substantially the point where the edge normally moves inwardly of the sheet.

14. In sheet glass apparatus, means for drawing a sheet from a mass of molten glass, upper and lower rolls arranged at each edge of the sheet and engaging the same, the lower roll being arranged at the formative portion of the edge and the upper roll being arranged at substantially the point where the edge normally moves inwardly of the sheet, and means for driving the upper roll in the

manner that it will have a peripheral speed relatively greater than that of the lower roll.

15. In sheet glass apparatus, means for drawing a sheet from a mass of molten glass, a rotatable bending member for deflecting said sheet from one plane to another, a plurality of pairs of rolls arranged at each edge of the sheet and engaging the same, the pair of rolls adjacent the bending member being driven at a speed intermediate the speed of the said bending member and the other rolls.

16. In sheet glass apparatus, means for drawing a sheet from a mass of molten glass, a rotatable bending member for deflecting said sheet from one plane to another, upper and lower pairs of rolls arranged at each edge of the sheet and engaging the same, the upper rolls being driven at a speed intermediate the speed of the lower rolls and bending member.

17. In sheet glass apparatus, means for drawing a sheet from a mass of molten glass, a rotatable bending member for deflecting said sheet from one plane to another, upper and lower pairs of rolls arranged at each edge of the sheet and engaging the same, and means for retarding the pairs of rolls in a manner that the peripheral speed of the upper rolls will be relatively greater than that of the lower rolls and relatively less than that of the bending member.

18. In sheet glass apparatus, means for drawing a sheet from a mass of molten glass, a rotatable bending member for deflecting said sheet from one plane to another, upper and lower pairs of rolls arranged at each edge of the sheet and engaging the same, the lower rolls being arranged at the formative portion of the edge and the upper rolls being arranged at substantially the point where the edge normally moves inwardly of the sheet, and means for driving the upper rolls in a manner that they will have a relatively greater peripheral speed than that of the lower rolls and relatively less peripheral speed than the bending member.

Signed at Charleston, in the county of Kanawha and State of West Virginia, this 10th day of May, 1924.

JOHN L. DRAKE.